# EUROPEAN PATENT SPECIFICATION

(11) **EP 2 050 845 B1**
(45) Date of publication and mention of the grant of the patent: **12.01.2011**
(21) Application number: 08166318.9
(22) Date of filing: 10.10.2008
(51) Int. Cl.: D02G 3/40, D03D 15/06

(54) **Process for the production of a fabric made of super-extra-fine yarns of high-quality fibres, which may not otherwise be produced industrially**
Verfahren zum Herstellen eines Stoffes aus extradünnem Garn aus hoch qualitativen Fasern, der ansonsten nicht industriell hergestellt werden könnte
Procédé de fabrication d'une étoffe à partir de fils super-extra fins de fibres de grande qualité, ne pouvant pas être autrement produit industriellement

(30) Priority: 19.10.2007 IT MI20072029
(43) Date of publication of application: 22.04.2009
(73) Proprietor: Geraldini, Jacopo, 20122 Milano (IT)
(72) Inventor: Geraldini, Jacopo, 20122 Milano (IT)
(74) Representative: Mittler, Enrico

(56) References cited:
- EP-A- 0 636 716
- EP-A- 1 061 162
- EP-A- 1 245 706
- CN-A- 1 259 596
- CN-A- 1 431 345
- GB-A- 775 387

## Description

The present invention relates to a process for the production of a fabric made of super-extra-fine yarns of high-quality fibres, which are unable to be produced industrially.

Based on modern technologies, a fabric made of extra-fine yarns of high-quality animal fibres, such as, for example, pure cashmere yarns or an intimate blend of cashmere and silk or extra-fine wool, vicuna, angora, alpaca etc., may be produced with a yarn count that may reach a maximum fineness of about 100 dtex / 83 dtex.

As a matter of fact, the poor kinetic strength of these extra-fine yarns means that they are extremely difficult to be woven.

In some cases, as disclosed in EP-A-1245706 and EP-A-1061162 a solution has already been found involving the use of doubling techniques that allow to guarantee a sufficient kinetic strength on the loom. This allows to produce fabrics in high-quality animal fibre yarns which may reach the fineness level described above, but may not exceed it.

CN-A-1431345 discloses a technology for producing high count worsted cloth by mixed spinning low temp water soluble polyvinyl and wools or crossed uniting polyvinyl with cotton yarn, muslin, silk and wool.

GB-A-775387 discloses a process for producing a yarn in which animal fibres are spun together with synthetic soluble fibres which are then removed by a solvent.

The object of the present invention is now to provide a process which allows to produce fabrics made of high-quality animal fibre yarns which are super-extra-fine, i.e. yarns having a higher degree of fineness, not currently available commercially, able to reach a yarn count of 33 dtex and finer.

In view of this object, the process according to the present invention includes the following steps:
a. spinning blended yarns consisting of an intimate blend of high-quality animal fibres and water-soluble synthetic fibres;
b. doubling said blended yarns with respective water-soluble synthetic yarns;
c. weaving the doubled yarns;
d. dissolving said water-soluble synthetic fibres and said water-soluble synthetic yarns by means of a slightly acidic aqueous solution brought to the temperature required for the dissolution to obtain a fabric consisting of yarns of pure animal fibres having a count lower than 55 dtex.

The starting blended yarns may consist of an intimate blend of very-high-quality animal fibres (e.g. pure cashmere or an intimate blend of 80% cashmere and 20% silk) and water-soluble fibres, not necessarily with an extra-fine yarn count, the latter in a varying percentage between a minimum of 5% and a maximum of 95% depending on the final yarn count of the desired super-extra-fine yarn, as well as on the specific characteristics of the desired type of fabric (particularly in terms of "feel"). The above-mentioned super-extra-fine yarns may be single ply or double ply.

The expression "water-soluble synthetic yarns" refers to synthetic-fibre yarns that may dissolve in a slightly acidic aqueous solution brought to the temperature required for the dissolution. They preferably, but not necessarily, have the same yarn count as the extra-fine yarns.

Doubling may be achieved through two different procedures concerning the direction of twist to be performed during the step of coupling, with the main reference direction being that of the extra-fine yarn having animal fibres. The direction of twist of the yarn entirely made of water-soluble material is actually completely uninfluential and irrelevant.

Depending on the desired final product, the following two assumptions are possible:
- doubling the water-soluble yarn with the blended yam(s), with a low number of twists, in the opposite direction to the twist of the blended yarn(s). This allows to obtain a final product which is particularly soft, fluffy and delicate;
- doubling the water-soluble yarn, with a low number of twists, in the same twist direction as the blended yarn(s). This allows to obtain a final product which is particularly dynamic, fresh and less subject to the problems of 'pilling'.

By way of mere example, an extra-fine yarn made of a blend of fibres in the proportions of 50% cashmere (WS) and 50% water-soluble fibres (PVA) is considered, with a yarn count of 111 dtex, which is doubled with a yarn entirely made of PVA, with the same yarn count as the blended yarn.

A doubled yarn with a yarn count of 111 dtex multiplied by 2 and an overall composition of 25%WS - 75%PVA is thus obtained, which will be employed in the normal step of weaving to create a coarse fabric.

The coarse fabric is then subjected to a step of scouring dyeing, which includes an operation of dissolving or melting the water-soluble fibres (based on the procedures required by/provided for the specific type of PVA), in order to be able to obtain a final fabric entirely made of 100% WS, with a final super-extra-fine yarn count of 55 dtex, which is absolutely impossible to be achieved through the currently known techniques.

The above-mentioned super-extra-fine yarn count may be simply calculated beforehand from the step of composing the starting extra-fine yarn blend; in the above described case, since the starting yarn count of 111 dtex and the fibre blend compound of 50% WS and 50% PVA are known, once the said 50% PVA aliquot has dissolved, the final yarn count for the fabric (100%WS) will be half the initial yarn count, i.e. 55 dtex, which is well beyond the fineness parameters which are currently possible or imaginable.

As previously mentioned, the variability of the parameters concerning the percentage of PVA and animal fibres in the blended yarn, may also be detected for specific needs, such as those of 'feel'.

In fact, a hypothetical yarn count of 55 dtex may be achieved either by exactly applying the fineness parameters and/or composition percentages described above, or by means of a similar procedure involving however the use of a lower extra-fine yarn count, equivalent to 222 dtex, along with a composition of 25% WS and 75% PVA. However, the product thus obtained, although it also has a yarn count of 55 dtex, might display a slightly different "feel", naturally as desired result.

It will be apparent that, based on the composition aliquots of the extra-fine yarn, the starting yarn count thereof might also be well below the levels which are considered fine and/or extra-fine.

The accompanying drawings show two practical embodiments of the process according to the present invention. Specifically:
figure 1 shows an extra-fine yarn of high-quality animal fibres, in particular extra-fine cashmere fibres and possibly silk fibres, in an intimate blend with water-soluble fibres, doubled in the opposite direction with a yarn of water-soluble synthetic fibres, specifically polyvinyl fibres;
figure 2 shows a portion of a coarse fabric obtained by weaving doubled yarns such as those in figure 1;
figure 3 shows the same portion of fabric after the synthetic fibre yarns have been dissolved;
figure 4 shows an extra-fine yarn of high-quality animal fibres, in particular extra-fine cashmere fibres and possibly silk fibres, in an intimate blend with water-soluble fibres, doubled in the same direction with a yarn of water-soluble synthetic fibres, specifically polyvinyl fibres;
figure 5 shows a portion of a coarse fabric obtained by weaving doubled yarns such as those in figure 1;
figure 6 shows the same portion of fabric after the synthetic fibre yarns have been dissolved;
figure 7 shows an example of doubling an extra-fine two-ply yarn with a water-soluble synthetic fibre yarn.
Figure 8 shows a different kind of representation of the doubled yarns of figure 7.

The starting blended yarn, indicated by numeral 1, was created by traditional spinning with a Z-twist, preferably with 850 turns per linear metre.

The yarn 1 is then doubled with a yarn 2 having substantially the same yarn count, also having a Z-twist, preferably with 850 turns per linear metre, consisting of the so-called 'water-soluble' synthetic fibres, i.e. fibres which dissolve in a slightly acidic aqueous solution at the appropriate temperature, specifically polyvinyl material (PVA). The yarn 2 may be made of fibres woven with a cotton-type cut (thus having a discontinuous nature).

Doubling is carried out with an S-twist, preferably with 340 turns per linear metre, so as to obtain a correct final balancing of the doubled yarn, indicated by numeral 3 in figure 1.

As shown in figure 2, an appropriate number of doubled yarns 3 is then subjected to a traditional warp and weft weaving (or on a circular Jersey-type machine), in which the polyvinyl yarns 2 serve as a support to allow the blended yarns 1 to be woven, which may not otherwise be woven industrially.

The coarse fabric thus obtained, which may have any cloth-, twill- or jacquard-type weave, clearly has the same composition as the doubled yarn 3.

Such a coarse fabric is then subjected to a step of scouring dyeing, whrein it is immersed in an aqueous solution of about 50 litres per 1 kg of polyvinyl with a slightly acidic pH (about 4.5) at a dissolution temperature in the range between 30°C and 100°C (depending on the nature of the PVA yarn).

The PVA yarn 2 and any similar water-soluble fibres present in the yarn 1 are thus eliminated by dissolving or melting, leaving a final fabric (fig. 3) exclusively consisting of yarns 1' with a super-extra-fine yarn count (even up to 33 dtex) made of high-quality animal fibres only (pure cashmere or cashmere and silk), which would otherwise have been impossible to be achieved by means of traditional techniques.

In virtue of the doubling S-twist in a direction opposite to that of the single yarns 1 and 2, after the water-soluble material has dissolved, the remaining yarn 1' has a twist equivalent to the algebraic sum of the spinning (850 Z) and doubling (340 S) twists, i.e. in the example shown equivalent to 510 Z. In virtue of this reduced twist, the resulting fabric is therefore extremely soft, as well as with an extra-fine yarn count.

Alternatively, the doubling operation may be carried out by a doubling Z-twist, i.e. in the same direction as that of the yarns 1, as shown in figures 4 and 5.

In such a case, after the water-soluble yarns 2 and the water-soluble fibres which make up the yarns 1 have melted, the remaining yarn 1' has a twist equivalent to the sum of the spinning and doubling twists, i.e. in the example shown equivalent to 1190 Z, but this is still low enough to make the final fabric soft, while considerably reducing the "pilling" effect.

Finally, as shown in figures 7 and 8, a water-soluble yarn 2 may be doubled (in a clockwise or anticlockwise direction) with two blended yarns or a two-ply yarn 1. After the weaving, a coarse fabric made of three-ply warp and weft yarns is obtained ,which, once the water-soluble yarns have been dissolved, will become a finished fabric with super-extra-fine yarns completely identical to that shown in figures 3 and 6, but with two-ply yarns.

## Claims

1. A process for the production of a fabric made of yarns of pure animal fibres having a count lower than 55 dtex , **characterised in that** it includes the following sequence of steps:
a. spinning blended yarns (1) consisting of an intimate blend of high quality animal fibres and water-soluble synthetic fibres;
b. doubling said blended yarns (1) with respective water-soluble synthetic yarns (2);
c. weaving the doubled yarns (3);
d. dissolving said water-soluble synthetic fibres and said water-soluble synthetic yarns (2) by means of a slightly acidic aqueous solution at the temperature required for the dissolution to obtain a fabric consisting of yarns (1') of pure animal fibres having a count lower than 55 dtex.

2. A process according to claim 1, **characterised in that** said animal fibres are pure cashmere.

3. A process according to claim 1, **characterised in that** said animal fibres are cashmere and silk.

4. A process according to anyone of the claims 1-3, **characterised in that** the doubling is carried out with blended yarns (1) and water-soluble synthetic yarns (2) having the same yarn count.

5. A process according to anyone of the claims 1-4, **characterised in that** the doubling is carried out with a twist in an opposite direction to that of the blended yarns (1).

6. A process according to claim 5, **characterised in that** the doubling is carried out with an S-twist.

7. A process according to anyone of the claims 1-4, **characterised in that** the doubling is carried out with a twist in the same direction as that of the blended yarns (1).

8. A process according to claim 7, **characterised in that** the doubling is carried out with a Z-twist.

9. A process according to anyone of the preceding claims, **characterised in that** said blended yarns (1) are single-ply.

10. A process according to anyone of the preceding claims 1-8, **characterised in that** said blended yarns (1) are double-ply.

## Patentansprüche

1. Verfahren zur Herstellung eines Gewebes, das aus Garnen reiner Tierfasem mit einer Zahl, die niedriger als 55 dtex ist, gefertigt ist, **dadurch gekennzeichnet, dass** es die folgende Ablauffolge von Schritten enthält:
a. Spinnen gemischter Garne (1), die aus einer vertrauten Mischung von Tierfasern hoher Qualität und wasserlöslichen, synthetischen Fasern besteht;
b. Verdoppeln der gemischten Garne (1) mit jeweiligen wasserlöslichen, synthetischen Garnen (2);
c. Weben der verdoppelten Garne (3);
d. Auflösen der wasserlöslichen, synthetischen Fasern und der wasserlöslichen, synthetischen Garne (2) mittels einer etwas säurehaltigen, wasserartigen Lösung bei der Temperatur, die für die Auflösung erforderlich ist, um ein Gewebe zu erhalten, das aus Garnen (1') aus reinen Tierfasern mit einer Zahl, die niedriger als 55 dtex ist, besteht.

2. Verfahren nach Anspruch 1, **dadurch gekennzeichnet, dass** die Tierfasern reines Kaschmir sind.

3. Verfahren nach Anspruch 1, **dadurch gekennzeichnet, dass** die Tierfasern Kaschmir und Seide sind.

4. Verfahren nach einem der Ansprüche 1-3, **dadurch gekennzeichnet, dass** das Verdoppeln mit gemischten Garnen (1) und wasserlöslichen, synthetischen Garnen (2) mit derselben Garnzahl ausgeführt wird.

5. Verfahren nach einem der Ansprüche 1-4, **dadurch gekennzeichnet, dass** das Verdoppeln mit einer Drehung in einer entgegengesetzten Richtung zu derjenigen der gemischten Garne (1) ausgeführt wird,

6. Verfahren nach Anspruch 5, **dadurch gekennzeichnet, dass** das Verdoppeln mit einer S-Drehung ausgeführt wird.

7. Verfahren nach einem der Ansprüche 1-4, **dadurch gekennzeichnet, dass** das Verdoppeln mit einer Drehung in derselben Richtung wie derjenigen der gemischten Garne (1) ausgeführt wird.

8. Verfahren nach Anspruch 7, **dadurch gekennzeichnet, dass** das Verdoppeln mit einer Z-Drehung ausgeführt wird.

9. Verfahren nach einem der vorangehenden Ansprüche, **dadurch gekennzeichnet, dass** die gemischten Garne (1) einlagig sind.

10. Verfahren nach einem der vorangehenden Ansprüche 1-8, **dadurch gekennzeichnet, dass** die gemischten Garne (1) zweilagig sind.

## Revendications

1. Procédé pour la production d'un tissu fait en fils de fibres animales pures ayant un titre inférieur à 55 dtex, **caractérisé en ce qu'**il comprend la séquence d'étapes suivantes:
a. filage de fils mélangés (1) constitués d'un mélange intime de fibres animales de haute qualité et de fibres synthétiques solubles dans l'eau ;
b. doublage desdits fils mélangés (1) avec des fils synthétiques solubles dans l'eau (2) respectifs ;
c. tissage des fils doublés (3);
d. dissolution desdites fibres synthétiques solubles dans l'eau et desdits fils synthétiques solubles dans l'eau (2) au moyen d'une solution aqueuse légèrement acide à la température requise pour la dissolution afin d'obtenir un tissu constitué de fils (1') de fibres animales pures ayant un titre inférieur à 55 dtex.

2. Procédé selon la revendication 1, **caractérisé en ce que** lesdites fibres animales sont en cachemire pur.

3. Procédé selon la revendication 1, **caractérisé en ce que** lesdites fibres animales sont en cachemire et en soie.

4. Procédé selon l'une quelconque des revendications 1 à 3, **caractérisé en ce que** le doublage est effectué avec des fils mélangés (1) et des fils synthétiques solubles dans l'eau (2) ayant le même numéro de fil.

5. Procédé selon l'une quelconque des revendications 1 à 4, **caractérisé en ce que** le doublage est effectué avec une torsion dans une direction opposée à celle des fils mélangés (1).

6. Procédé selon la revendication 5, **caractérisé en ce que** le doublage est effectué avec une torsion S.

7. Procédé selon l'une quelconque des revendications 1 à 4, **caractérisé en ce que** le doublage est effectué avec une torsion dans la même direction que celle des fils mélangés (1).

8. Procédé selon la revendication 7, **caractérisé en ce que** le doublage est effectué avec une torsion Z.

9. Procédé selon l'une quelconque des revendications précédentes, **caractérisé en ce que** lesdits fils mélangés (1) sont simple brin.

10. Procédé selon l'une quelconque des revendications 1 à 8, **caractérisé en ce que** lesdits fils mélangés (1) sont double brin.
